

## UNITED STATES PATENT OFFICE.

ANSON GARDNER BETTS, OF KINDERHOOK, NEW YORK.

## ART OF SMELTING MANGANESE.

No Drawing.

Application filed November 23, 1925. Serial No. 70,819.

This invention relates to the recovery of manganese from ores, by smelting, particularly to its recovery from ores and earthy material containing manganese, of comparatively low grade.

The principal object of this invention is to extract manganese by smelting, at low cost, and thereby to utilize low grade manganeseiferous material now considered to be of no, or low value, as well as to recover when desirable certain by-products as may be noted from the following. Other objects will appear from the following description.

Hitherto, crude manganese metal, known as ferromanganese, or in lower grade known as spiegeleisen, the principal manganese metallic products, have in general only been successfully produced from ores that would be considered of exceptionally high grade, if applying to other metals as copper, lead or zinc, for example. The amount of high grade manganese ores, low in percentage of silica and deleterious ingredients, compared to lower grade materials still containing considerable percentages of manganese, is believed to be extremely limited in comparison, and also, at the present time, is mostly mined in regions of the earth which are very remote from the principal regions of consumption, i. e., the steel producing regions.

Manganese is the most abundant of the heavy metals, after iron, and the amount of lower grades of manganese ore, which ores would be considered of very good grade if they were ores of copper or lead, for example, is sufficient for all requirements, and not so remote from districts where manganese is consumed. As far as I know, these materials are not now being utilized for making ferromanganese, or spiegeleisen.

Such lower grade manganese material may be a mixture of manganese oxides and slaty or silicious material and dirt, and may contain considerable percentages of oxide of iron. Some of these materials are known as manganeseiferous iron ores, more or less silicious. There are slaty beds of manganeseiferous material in abundance, manganeseiferous clays containing nodules of manganese oxides and black soft manganese streaks not now saved in mining. There are deposits of rhodonite, silicate of manganese, carrying 20 or more percent of manganese, with much silica. There are large amounts of oxidized rhodonite, consisting of an intimate mixture of silica and manganese oxides, carrying 30%

or more of manganese. My present process is believed to be adapted to all of these materials when carrying sufficient manganese.

Naturally, the details of a process would be varied in treating such a variety of materials, while still operating on the same principle in respect of the manganese contents, the variations being such as would be applied by one skilled in the art, in view of the present disclosure, to properly provide for and take care of the other ingredients, and to utilize them as far as may be, for valuable by-products.

In the ordinary smelting of manganese, the cost of producing crude manganese metal, is greatly increased by the presence of even moderate amounts of silica, which is the chief ingredient in the average lower grade manganese material. Also, considerable manganese material otherwise of good or fair grade, is rendered of low value by the presence of considerable iron. The iron appears as an alloy of manganese and makes the manganese of less value and the cost of reducing iron in a manganese furnace is materially greater than the cost of reducing iron in an iron furnace, thus making a loss on the iron made, in addition.

In my process, instead of smelting the ore to produce crude metallic manganese alloyed with more or less iron, the less iron the better, and also containing carbon, I smelt the ores to produce as principal manganese product, a crude, fused sulphide of manganese, herein called a "matte" which separates separately from the reduced iron, and from the slag containing the silica and fluxes therefor, found in the materials used, and added specially as flux. This accomplishes the two principal objects, that is, separation from iron, and from silica, by a comparatively cheap process of wide application relatively to various grades and kinds of manganese materials. Of course, if the iron is present in the charge in relatively small amounts, it is not necessarily profitable, and in the process it is not necessary, to make a product of metallic melted iron, but the iron may be taken from the furnace as a sulphide alloyed with the manganese sulphide as a crude manganese and iron sulphide. However, in view of the amount of iron that is not objectionable in crude manganese, that is about 1 part of iron to 4 parts of manganese, it is preferable to make a separate product of iron, when iron is present in materially greater amounts,

and in the case of manganeseiferous iron ores, the recovery of the iron may be a considerable part of the value of the operation and process.

While in the present art of smelting manganese ores to crude manganese metal, very basic and expensive slags must be made, with high losses of manganese in the slag and expelled from the furnace as a fume, with very high temperatures, very expensively produced, these difficulties very largely disappear, in using my process, because the slag may be made more silicious and therefore cheaper, the operation can be carried out at much lower temperatures and therefore 15 much cheaper on that account, with largely increased output from a given furnace. It might be mentioned further, that the process provides opportunity to work manganese materials containing considerable phosphorus, as the melted iron collects the bulk 20 of the phosphorus and removes it from the manganese sulphide, beside which phosphorus may be made to go in the slag to some extent, under some conditions.

Obviously, this process requires sulphur to be present in the furnace charge, to produce the manganese as sulphide. Manganese ores that I am familiar with, do not contain sulphur in sufficient, or even in small 30 amounts. I accordingly introduce with the furnace charge a sulphur-bearing ingredient as a solid. It might be feasible to introduce sulphur as a vapor, by some means, and if so, such procedure would answer the requirements, but I regard that method as probably 35 impracticable. I may use, principally, iron or calcium sulphides, or equivalents of the latter. Calcium sulphate, gypsum or anhydrite, are equivalents of the latter, as in the furnace, calcium sulphate in presence of fuel, becomes converted into calcium sulphide. Other equivalents are the sulphides or sulphates of sodium, potassium, strontium or barium, but on account of the higher value of 40 the sulphates and sulphides of such elements other than calcium, I regard them more as equivalents chemically, than commercially, and in this description I shall only describe the use of the compounds of calcium in this 45 connection.

In one example of the process, a silicious manganese ore is smelted in a blast furnace with an iron pyrite or pyrrhotite ore, limestone or dolomite as flux for the silica and alumina, and coke for fuel and as reducing agent. The silicious and aluminous matters unite with lime and magnesia to form a slag. More or less sulphur may be expelled, particularly from bisulphide of iron, pyrite, 55 with the furnace gases but large amounts thereof unite with the manganese to form a fused, crude, manganese sulphide, or matte, while iron separates separately as melted iron. The separation of the iron, matte and 60 slag, will be well understood by furnacemen.

They may be tapped separately from the furnace, or may be drawn off together into a forehearth or auxiliary furnace in which they separate in layers, according to the different specific gravities, iron on the bottom, 70 matte in the middle, and slag on top, being tapped separately from the forehearth.

Chemically, the following reactions may be written by way of illustration, following the conventional way of representing processes in which chemical change take place.

Pyrite is decomposed at low temperatures, into sulphur and sulphide of iron. This will take place as the charge warms up and the sulphur burns off or is volatilized:



Reduction of manganese oxides to lower oxides, approximately represented as follows:



Reaction between manganese oxide and iron sulphide in presence of fuel for reduction, by one or both of the following



It is not necessary to write equations showing the formation of slag, largely or mainly of calcium silicate. Slag is a chemically indefinite material containing a mixture of oxides of bases and silica, fluxing each other into melted slag.

In another example of the process, the material to be smelted, beside containing manganese and earthy silicious matters, also contains iron oxides, so that the ore is a more or less silicious and impure iron-manganese ore, known as a "manganese" ore, meaning 100 manganeseiferous iron ore.

In this example, the process is identical with the foregoing example, except that the iron oxides are reduced by the agency of fuel, to metal, and the amount of iron produced, is thereby increased to the corresponding extent.

In another example, the formation of manganese sulphide, is, in whole or in part, brought about, by the use of calcium sulphide, which may be conveniently introduced as the 110 cheap and abundant native calcium sulphate, anhydrite or gypsum, the difference in the two being a mere difference in that gypsum contains water, about 21%. Sufficient fuel is allowed for, and contained in the charge, to effect the change of the calcium sulphate to calcium sulphide.

Calcium sulphide then reacts with manganese oxide, whether present in the hot charge as manganese oxide, or combined with silica, 125 as manganese silicate, producing as products, manganese sulphide, and calcium silicate dissolved in and being part of, the slag. The following equation may be written by way of illustration, although the practical process 130

lacks the chemical definiteness of a pure and a product of calcium sulphide, by substantially the chemical reaction:



5 It may be noted, that this reaction, does not produce any metallic iron, but only two products, manganese matte, and slag. If iron oxides are present in the furnace charge in large quantity, they are reduced by fuel, and 10 a product of iron also obtained, nevertheless.

In still another example of the process, the ore used contains oxides of iron and manganese, each in considerable amounts worth recovering as separate products, beside silicious 15 matter. It is obvious that the silicious matter requires a base to flux it into a slag, and lime in the standard and ordinary flux, sometimes in part replaced by magnesia by using dolomite instead of limestone. The lime for 20 making the slag, however, is not in this example, mainly supplied by the use of raw or burnt limestone, but in the shape of calcium sulphate. In the foregoing example, it has been pointed out that the calcium sulphate, 25 yields sulphur to make the manganese matte, beside furnishing calcium oxide for the slag, and in this example, the quantities are proportioned, as is readily done by one skilled in the art, so that the calcium sulphate doubly 30 performs the two functions of slag and matte maker, without requiring other flux, for the silica.

In a still further example, using calcium sulphate, the amount of silica present, is not sufficient, to combine with the lime of the 35 calcium sulphate to make the most desirable slag, and both iron sulphide and calcium sulphate are used, thereby cutting down the amount of lime to be slagged, and producing 40 more iron product.

Crude manganese sulphide is not a commercial product and would be worthless, if used directly, in making steel, where most of the manganese is consumed. It requires 45 to be converted into metal, or other manganese products. I prefer to do this, by mere oxidation of the sulphide in furnaces, with air, either at relatively low temperature, by the process known for other metals as "roasting", 50 or at higher temperatures, in the fused state, by blowing air through, in the process known as "Bessemerizing." In either case, the product is oxide of manganese, and sulphurous gases, which may be condensed and used as 55 sulphuric acid, by well known methods. Such oxide of manganese, practically free from silica, and relatively free from deleterious ingredients, is the ideal material for the production of crude or refined manganese metal 60 for its various uses.

Another method, which I may refer to, as it has some bearing on a phase of the process, consists in smelting manganese sulphide, 65 preferably in electric furnaces, with lime and carbon, producing crude manganese metal,

The calcium sulphide is valuable for the 70 process, as part of the smelting charge, beside which, any manganese sulphide contained therein, is merely returned to the process and not lost.

Broadly, the process of recovery consists 75 in smelting the ore with addition of sulphur in some practicable form, producing a fused manganese sulphide product and converting this into manganese metal.

Since, when iron sulphide ore, etc., is used 80 as the supplier of sulphur to produce manganese sulphide from the manganese of the manganese ore, etc., the iron thereof is recovered as metallic iron, in its preferred form the process gives an additional useful result, 85 the recovery of metallic iron from its sulphide, which is in general a very cheap or practically worthless material.

In the particularly preferred form, the 90 process includes the further step of converting the manganese sulphide to an oxide by oxidation and reducing the oxide to metallic manganese.

The process is applicable to slags containing manganese, produced in smelting processes. Some slags made in lead smelting carry considerable manganese and iron and have been thrown away and may be treated by my process. Also slags from ferromanganese furnaces, and other slags made in connection with iron smelting operations, may be worked for the manganese or manganese and iron contained therein.

The term "sulphur-introducing ingredient" used in the claims refers to iron or calcium sulphide or calcium sulphate as hereinbefore described, and equivalents, serving to supply the sulphur needed to produce manganese sulphide from the manganese oxide present in the manganese-bearing material 105 to be smelted for the production of manganese sulphide. This term would not include manganese sulphide as manganese sulphide would not have the property of introducing sulphur to other manganese, its affinity for 110 manganese being already satisfied.

What I claim as new and desire to secure by Letters Patent, is:

1. Process of recovering manganese from material containing manganese and silica 120 which consists in smelting said material with addition of a sulphur-introducing ingredient, producing fused manganese sulphide, and fused slag containing the silica of said material.

2. Process of recovering manganese from material containing manganese and silica which consists in smelting said material with addition of a sulphur-introducing ingredient, producing fused manganese sulphide, 130

fused metallic iron, and fused slag containing the silica of said material.

3. Process of recovering manganese from material containing manganese and silica which consists in smelting said material with addition of a sulphide other than of manganese, producing fused manganese sulphide, fused metallic iron, and fused slag containing the silica of said material.

10 4. Process of recovering manganese from material containing manganese and silica which consists in smelting said material with addition of iron sulphide, producing fused manganese sulphide, fused metallic iron, and fused slag containing the silica of said material.

15 5. Process of recovering manganese from material containing manganese and silica which consists in smelting said material with

addition of iron sulphide, producing fused manganese sulphide, fused metallic iron, and fused slag containing the silica of said material, and converting said manganese sulphide to manganese metal.

6. Process of recovering manganese from material containing manganese and silica which consists in smelting said material with addition of a sulphide other than of manganese, producing fused manganese sulphide, fused metallic iron and fused slag containing the silica of said material, converting said manganese sulphide to manganese oxide and reducing said manganese oxide to metallic manganese.

In testimony whereof I have hereto signed my name this 5th day of November, 1925.

ANSON GARDNER BETTS.